

## UNITED STATES PATENT OFFICE.

WILLETT C. PIERSON, OF CLEVELAND, OHIO.

## COMPOSITION FOR MATCH-HEADS.

1,138,146.

Specification of Letters Patent. Patented May 4, 1915.

No Drawing.

Application filed October 28, 1912. Serial No. 728,046.

*To all whom it may concern:*

Be it known that I, WILLETT C. PIERSON, a citizen of the United States of America, residing at Cleveland, in the county of Cuyahoga and State of Ohio, have invented certain new and useful Improvements in Compositions for Match-Heads; and I hereby declare the following to be a full, clear, and exact description of the invention, such as will enable others skilled in the art to which it pertains to make and use the same.

This invention relates to new and useful improvements in compositions for match heads.

The object of this invention primarily consists in providing a non-phosphorous composition for match-heads.

A further object of my invention is to provide a composition which can be cheaply manufactured and safely handled involving absolutely no danger to the health of the people employed in the manufacture and greatly minimizing the risk from explosion or combustion during the process of manufacture.

A further object of my invention is to provide a composition of this character which will be practically unaffected by climatic conditions in order that the manufacture of the said composition can be carried on without interruption due to unfavorable weather conditions and also that the completed match may keep in any climate without deterioration.

With these objects in view and with the intention of securing other advantages which will hereinafter appear, my invention consists in the composition hereinafter described in the specification and particularly pointed out in the claims.

In carrying out my process I take a predetermined quantity of a nitrated product preferably a nitrated carbohydrate and to this I add an oxygen supplying agent and some inert material which acts as a filler and abrasive. In order to obtain my nitrated product I have found that the following procedure gives very good results. I first take a quantity of a fibrous vegetable substance, preferably wood and veneer cut the same to the thickness of about one-sixteenth of an inch. I then treat the wood with a solution of sulfurous acid in water and heat sufficiently to dissolve the gum and other cementitious ingredients leaving the cellulose in an undissolved state. The cel-

lulose is then treated with nitric acid of 1.42 specific gravity and with excess of hot water and the cellulose is boiled until the whole is converted to pulp, water being added from time to time to replace that lost by evaporation. The nitrated product is then dried and pulverized, preferably by passing the same through a French Buhr grinding mill so that the pulverized material can pass through a hundred mesh screen. The nitrated product thus obtained I believe is nitrated cellulose.

In preparing the match-head composition I take a predetermined quantity of my nitrated product and add thereto a nitrate of some metal, such as silver nitrate, copper nitrate or lead nitrate, and also an oxidizing agent, a binder and a filler or abrasive.

In mixing my ingredients I proceed as follows:—To every twenty-four parts of the nitrated product I add one part of silver nitrate with sufficient water to dissolve the nitrate and saturate the whole mass which is then allowed to stand until thoroughly impregnated. The resulting product will have an acid reaction and must preferably be neutralized and to secure the neutralization thereof I treat the same with ammonia. The material after neutralization is slowly dried *in vacuo* and the resulting mass, in which no moisture should be present, is sealed in containers which will protect it from the action of light and air. The containers of course must be perfectly dry and to insure this they must be kept in an oven for two hours at a temperature of one hundred degrees centigrade. It may be here remarked that the nitrated cellulose after being treated with a metallic nitrate is exceedingly light in comparison to its bulk and a very small quantity by weight will be sufficient to dip a very large quantity of matches.

When the other materials have been prepared for mixing I take about twenty parts of the nitrated cellulose which has been treated with the metal nitrate and add thereto about ninety parts of potassium chlorate, six parts of bi-chromate of potash, fourteen parts of sulfur, eight parts of plaster of Paris, thirty-eight parts of ground glass, thirty-two parts of glue and two parts of free silver nitrate, making in all two hundred and ten parts. The match splints are dipped in the usual manner in this composition and a very firm head is formed thereon which will ignite very

readily and causes a quick combustion of the splint.

What I claim is,—

1. An igniting material containing a nitrated carbohydrate, a metallic nitrate, potassium chlorate, bi-chromate of potash, plaster of Paris, sulfur, powdered glass and glue.
- 5 2. An igniting material containing a nitrated cellulose, a metallic nitrate, potassium

chlorate, bi-chromate of potash, plaster of Paris, sulfur, powdered glass and glue.

In testimony whereof, I sign the foregoing specification, in the presence of two witnesses.

WILLETT C. PIERSON.

Witnesses:

B. C. BROWN,  
N. L. McDONNELL.

Copies of this patent may be obtained for five cents each, by addressing the "Commissioner of Patents.  
Washington, D. C."